

## UNITED STATES PATENT OFFICE

2,163,535

## THIOCARBONATED - CHLORALIPHATIC HYDROCARBONS AND METHOD OF MAKING SAME

Henry G. Berger, Woodbury, Robert C. Moran, Wenonah, and Francis M. Seger, Pitman, N. J., assignors to Socony-Vacuum Oil Company, Incorporated, New York, N. Y., a corporation of New York

No Drawing. Application December 21, 1938,  
Serial No. 246,996

17 Claims. (CL. 260—455)

This invention has to do in a general way with new chemical compositions or reaction products and is more particularly related to a novel group or class of reaction products which we have found 5 to be especially valuable as addition agents for lubricants in that they materially increase the load-carrying capacity of the lubricant carrying medium to which they are added and at the same time they do not possess the undesirable properties present in many of the so-called extreme 10 pressure agents heretofore developed.

Although the product or class of products contemplated by the present application has been developed especially for use as additive agents for 15 extreme pressure lubricants, it is to be understood that other uses may become apparent to those skilled in the art and that the present application is directed to the reaction product and is not to be construed as limited in any way by this 20 preferred field of usefulness since lubricant compositions containing the reaction products contemplated by the present application have been disclosed and claimed in our copending applications Serial No. 123,846, filed February 3, 1937, and Serial No. 200,910, filed April 8, 1938, of which the present application is a continuation in part.

The products of the present application may be broadly identified as "thiocarbonated-chloraliphatic hydrocarbons", or as polychlorinated hydrocarbons in which the more reactive part of 30 the combined chlorine has been replaced by a thiocarbonate group.

The preferred procedure which may be followed in synthesizing the products of our invention involves 35 substantial chlorination of an aliphatic compound or predominantly aliphatic material, such as petroleum naphtha, followed by the reaction of the chlorinated material with an alkali or alkaline earth metal salt of an alkyl thiocarbonic acid in such proportions and under such 40 conditions that only a part of the chlorine (that is, the more reactive chlorine) is replaced by the alkyl thiocarbonate group. The reaction product thus obtained is an aliphatic or predominantly 45 aliphatic hydrocarbon material containing chlorine and thiocarbonate groups in chemical combination with the aliphatic hydrocarbon. This product may be blended in minor proportions with a mineral oil lubricant to effect substantial 50 improvement in the load-carrying capacity of the oil without impairing the color of the oil and without causing corrosion of containers in which it is stored. It is clearly distinguished from products such as might be obtained by the chlorination 55 of a dialkyl thiocarbonate (such as ethyl

ethyl xanthate), which when blended with a mineral oil lubricant is highly corrosive to containers and causes substantial deterioration in the color of the oil. The product of our invention contains residual chlorine in addition to the thiocarbonate group and is thus clearly distinguished from a product such as that disclosed in U. S. Patent No. 1,491,021, wherein oxy-normal-butyl thiocarbonic acid disulfide is obtained by chlorinating sodium butyl dithiocarbonate. 10

We have found that for the purpose of synthesizing the products of the present invention, which have the property of improving the load-carrying ability of lubricants, the aliphatic material can be chosen from a relatively wide range 15 of aliphatic compounds or hydrocarbon materials which are predominantly aliphatic in nature. The range of aliphatic materials which may be chlorinated as the starting material has been found to extend from ethane to petroleum wax, 20 the former being a compound containing two carbon atoms and the latter being a predominantly aliphatic material corresponding to a compound having substantially twenty carbon atoms. 25 We have found, however, that the extremely short chain compounds represented by polychlorethanes and the extremely long chain compounds represented by chlorinated petroleum wax are somewhat more difficult to react and are somewhat less efficient in their final composition as 30 "extreme pressure agents" than hydrocarbons of an intermediate range, and for that reason preference is given to aliphatic materials within the range of from about five to about fifteen carbon atoms, particular preference being given to petroleum naphtha, a hydrocarbon material predominantly aliphatic in nature corresponding to a compound having about ten carbon atoms. 35

In the chlorination step the aliphatic material is chlorinated to such an extent that the final 40 chlorinated product corresponds to a polychlor compound, and in the case of petroleum naphtha the chlorination is preferably carried to a point at which the product has an average composition corresponding to a tetrachloronaphtha. In general it may be said that chlorination should be carried to the point at which the chlorine content is from about forty per cent to about sixty per cent, although materials of lower and higher chlorine content may be used, depending upon 45 the aliphatic constituent. 50

The thiocarbonate group which is used to replace a part of the chlorine is, as has been indicated above, derived from an alkali or alkaline earth metal salt of a thiocarbonic acid, preferably

an alkyl thiocarbonic acid. The thiocarbonate radical may be a mono-, di-, or tri-thiocarbonate, but in general preference is given to the dithiocarbonate (xanthate) compounds characterized by the divalent group ( $OCS_2$ ). The trithiocarbonate type of compounds characterized by the divalent group ( $CS_3$ ) have also been prepared and have been found to form effective extreme pressure agents when reacted with the chlorinated aliphatic material, but from the standpoint of odor and cost preference is given to products in which the thiocarbonate constituent is a xanthate (divalent  $OCS_2$ ) group.

As to the alkyl substituents in the thiocarbonate or xanthate groups which are substituted in the chlorinated aliphatic material, it is preferable for the formation of products adapted for use as oil-improving agents that such substituents be derived from aliphatic compounds of relatively low molecular weight. There is no particular advantage to be gained by having a long chain alkyl group in the xanthate or thiocarbonate substituent from the standpoint of solubility, etc., and the lower molecular weight alkyl groups give a finished product in which the content of chlorine and characterizing divalent thiocarbonate groups ( $O_2CS$ ,  $OCS_2$  or  $CS_3$ ) is somewhat more highly concentrated.

As examples of the thiocarbonate or xanthate materials which may be reacted with chlorinated aliphatic materials to provide extreme pressure agents of the type contemplated by this invention, we may use sodium or potassium methyl, ethyl, benzyl, butyl or amyl xanthates or the corresponding mono- or tri-thiocarbonates.

It is highly important, as stated above, that the proportions of reactants used and the conditions of reaction be controlled so that the final product contains both chlorine and thiocarbonate characterizing groups in chemical combination with the aliphatic hydrocarbon material. The relative amounts of chlorine and sulfur, or, more specifically, of chlorine and thiocarbonate characterizing groups, in the finished product may be varied over a relatively wide range, but in general it may be said that the finished product should preferably be one which contains from about twenty-five to forty per cent chlorine and from about seven to fifteen per cent sulfur. Expressing the sulfur content as the equivalent amount of characterizing thiocarbonate groups present in the product, such preferred products are more accurately identified as containing from about ten per cent to about twenty-two per cent characterizing dithiocarbonate or xanthate (divalent  $OCS_2$ ) groups or from about seven per cent to about seventeen per cent characterizing trithiocarbonate (divalent  $CS_3$ ) groups. For general purposes it may be said that the characterizing thiocarbonate group content is preferably from about seven per cent to about twenty-two per cent.

The reaction between the chlorinated aliphatic material and the alkali thiocarbonate is preferably carried out in the presence of a relatively low boiling point solvent. For convenience in reaction and purification the solvent is preferably one in which the chlorinated aliphatic material and the reaction product are highly soluble but in which the alkali thiocarbonate and the alkali chloride are of low solubility. As an example of such a solvent we have found acetone to be highly satisfactory, although other solvents, such as methyl ethyl ketone, may be used. Alcohols may also be used as solvents in this reaction. Sol-

vents such as acetone and methyl ethyl ketone are particularly desirable since they permit the reaction to proceed but tend to precipitate residual alkali thiocarbonate and chloride, thus permitting the process to be performed and the product substantially purified all in one step.

The general preferred procedure followed in effecting the replacement of the more highly reactive chlorine in chlorinated aliphatic materials with the thiocarbonate group is to dissolve the chlorinated aliphatic material in the solvent and add the alkali alkyl thiocarbonate in an amount sufficient to give a product having the desired chlorine and sulfur ratio. Under the conditions of reaction which we employ we have prepared materials using from about one-fourth to about twice as much alkali thiocarbonate (xanthate) as chlornaphtha. The preferred ratio, however, is a weighted amount of alkali thiocarbonate corresponding to from about forty per cent to about seventy per cent of the weight of the chlornaphtha used. It will be understood, of course, that these ratios vary with other chlorinated aliphatic materials, depending upon their hydrocarbon and chlorine content, and should also take into consideration the alkyl substituent which is attached to the characterizing thiocarbonate group.

The procedure to be followed in the synthesis of the products contemplated by this invention will be best appreciated from the following examples:

#### Example I

As stated above, the preferred products contemplated by this invention are those obtained by replacing a part of the chlorine in chlorinated petroleum naphtha with an alkyl xanthate group. These materials are preferred to others of this general class of materials because of their ease of synthesis, their cost, etc. An exemplary procedure for preparing such a product, which we may term "chlornaphtha-xanthate reaction product", a "xanthated chlornaphtha" or "xanthochlornaphtha", is as follows:

A chlorinated naphtha was first prepared by chlorinating petroleum naphtha (Stoddard solvent) until it contained about fifty-four per cent by weight of chlorine. Twenty parts of the chlornaphtha were dissolved in about fifty parts of acetone and placed in a reaction vessel heated by a water jacket and equipped with stirrer and reflux condenser. To this solution twelve parts of potassium ethyl xanthate were added and the mixture held at boiling temperature with stirring under reflux for about two hours. The resulting mixture was cooled to room temperature, filtered, and the filtrate subjected to distillation to remove the acetone. After removal of the acetone the product was washed to remove potassium salts and was dried and filtered. The finished product obtained by the foregoing procedure, which for purpose of description herein may be termed "chlornaphtha-xanthate reaction product" or "chlornaphtha-ethyl xanthate reaction product" was a dark brown liquid containing about twelve per cent sulfur, or more specifically about seventeen per cent of the characterizing xanthate (divalent  $OCS_2$ ) group, and thirty-seven per cent chlorine.

Variation in xanthate and chlorine content of the reaction product can be obtained by varying the degree of chlorination of the naphtha; by varying the amount of alkali xanthate used; by varying the hydrocarbon substituent in the alkali xanthate; and by varying the time of reaction.

of the chlornaphtha and alkali xanthate. Thus products of widely varying chlorine and xanthate content are readily possible. In general, as indicated above, we prefer a product containing from about ten per cent to about twenty-two per cent of the characterizing xanthate group and from about twenty-five per cent to about forty per cent chlorine.

In ten per cent concentration in mineral lubricating oil a chlorine-and-xanthate-substituted naphtha obtained as a product from a synthesis such as is described above produces excellent extreme pressure lubricants, passing in a satisfactory manner the usual evaluation tests used in the art. Actual gear tests show the blends to have good extreme pressure properties without any tendency to form sludge and without corrosive action towards the steel parts or towards containers.

In addition to a product of the type described above, which is obtained by the reaction of chlorinated petroleum naphtha and potassium ethyl xanthate and which contains residual chlorine and the characterizing xanthate (divalent  $OCS_2$ ) groups, we have prepared numerous other products of this general type in which:

(a) Alkyl xanthates other than the ethyl xanthate group are substituted for the more highly reactive chlorine in chlornaphtha;

(b) Chlorinated aliphatic materials other than chlornaphtha are used as the starting material; and

(c) Thiocarbonate groups other than the xanthate group are substituted for the more highly reactive chlorine in chlorinated aliphatic material.

Compounds or materials of these other types are illustrated by the following additional examples:

#### Example II

One hundred parts of chlornaphtha (chlorinated Stoddard solvent of forty-nine per cent chlorine content) were reacted with fifty-two parts of potassium methyl xanthate, using acetone as a solvent and following the same general procedure described above, except that the mixture was refluxed for one hour. The product obtained, which we may term "chlornaphtha-methyl xanthate reaction product", contained 32.45 per cent chlorine and 9.79 per cent sulfur (about fourteen per cent of the characterizing xanthate group). A mineral oil containing ten per cent of this product passed the 30,000 pound load limit in the Almen pin test and showed a load limit of 370 pounds at 755 R. P. M. in the S. A. E. test.

#### Example III

251 parts of chlornaphtha (chlorinated Stoddard solvent of forty-nine per cent chlorine content) and 120 parts of potassium butyl xanthate were reacted in acetone in the same manner as described in Example II to give a product ("chlornaphtha-butyl xanthate reaction product") containing 28.6 per cent chlorine and about thirteen per cent of the characterizing xanthate (divalent  $OCS_2$ ) group. This product in a ten per cent concentration in mineral oil passed the Almen pin test at 30,000 pounds and showed a load limit of 335 pounds at 755 R. P. M. in the S. A. E. test.

#### Example IV

Two hundred twenty-six parts of chlorinated petroleum wax having a chlorine content of 50.42

per cent were reacted with 200 parts of potassium ethyl xanthate in the presence of acetone with refluxing for two hours to obtain a product ("chlornaphtha-ethyl xanthate reaction product") containing 37.58 per cent chlorine and about 13 per cent of the characterizing xanthate group. A 10 per cent admixture of this product with mineral oil showed a load limit of 17,000 pounds in the Almen pin test and of 425 pounds at 755 R. P. M. in the S. A. E. test.

10

#### Example V

Eighty-four parts of tetrachlorethane were reacted with 80 parts of potassium ethyl xanthate in the presence of denatured alcohol as a solvent, the reaction mixture being refluxed for two and one-half hours to obtain a product containing 54.3 per cent chlorine and about 15.9 per cent of the characterizing xanthate group. This product in 10 per cent admixture with mineral oil showed a load limit in the Almen pin test of 9,000 pounds and in the S. A. E. test of 230 pounds at 755 R. P. M.

15

20

25

#### Example VI

One hundred forty parts by weight of dichlorpentanes and 70 parts by weight of potassium ethyl xanthate in the presence of acetone as a solvent were refluxed for 1½ hours to yield a "chlorpentane-ethyl xanthate reaction product" containing about 27.6 per cent chlorine and about 19.3 per cent of the characterizing xanthate group. A ten per cent blend of this reaction product in a mineral oil of 80-90 seconds S. U. viscosity at 210° F. showed a load limit of 12,000-14,000 pounds in the Almen test and of 345 pounds at 1000 R. P. M. in the S. A. E. test.

30

35

40

#### Example VII

As previously stated, the extreme pressure ingredients contemplated herein as new compositions of matter include products obtained by the chemical substitution of part of the chlorine in a chlorinated aliphatic material with other thiocarbonate groups than the alkyl xanthate (dithiocarbonate) groups discussed in the foregoing examples. To illustrate the preparation of "chlornaphtha-alkyl trithiocarbonate reaction products" the following procedure may be used:

Petroleum naphtha (Stoddard solvent) was chlorinated by bubbling chlorine gas therethrough until it contained about fifty-two per cent by weight of chlorine. Two hundred twenty-five parts by weight of the chlornaphtha were then admixed with about 400 parts of acetone and 100 parts of potassium amyl trithiocarbonate. The mixture was refluxed with stirring on a water bath by heating for about one and a half hours, after which it was cooled and filtered to remove the potassium chloride. The acetone was removed by distillation, after which benzol was added and distilled off to insure removal of water from the product. The resulting product was a bright liquid soluble in oil, and a typical analysis showed a chlorine content of 35 per cent and a sulfur content of about 10 per cent, or more specifically a trithiocarbonate (divalent  $CS_2$ ) content of about 11.2 per cent. As in the xanthate product, the proportion of chlorine and the proportion of the characterizing trithiocarbonate group in such reaction product may be varied by choice of reactants and proportions used. The nature of the alkyl radical in the alkali trithiocarbonate may be varied. It will also be understood that in all of the foregoing representative reactions that the

45

50

55

60

65

70

75

alkali metal may be either sodium or potassium.

This trithiocarbonate product ("chlornaphtha-alkyl trithiocarbonate reaction product"), when blended in 10 per cent concentration with a mineral oil of 80-90 seconds Saybolt Universal viscosity at 210° F., passed the load limit of 30,000 pounds in the Almen pin test and gave a load limit of 390 pounds at 1000 R. P. M. in the S. A. E. test.

10

*Example VIII*

As a further example illustrating the synthesis of "chlornaphtha-alkyl trithiocarbonate reaction products" for use as extreme pressure ingredients, we have condensed chlorinated petroleum naphtha with a commercial product marketed under the trade name of "Floto". This material, which was used in place of the potassium amyl trithiocarbonate described in Example VII, is made from a mixture of refinery mercaptans and is a mixed sodium trithiocarbonate. The material is predominantly sodium ethyl trithiocarbonate, but the alkyl substituent probably ranges from methyl to amyl. The synthesis of the chlornaphtha trithiocarbonate prepared from this material followed the same procedure outlined above in Example VI, using 100 parts of chlorinated naphtha and 20 parts of Floto and 200 parts of acetone. The finished product contained 36.4 per cent chlorine and 7.1 per cent sulfur, or more specifically such product contained 8 per cent of the characterizing trithiocarbonate (divalent  $CS_3$ ) group.

*Example IX*

In the commercial production of "xanthated chlornaphtha" the procedure has been varied slightly from that described in Example I, the preferred method for commercial scale production being carried out as follows:

Stoddard solvent is chlorinated by first adding 1 per cent by weight of  $PCl_3$  and then bubbling chlorine gas therethrough at a temperature of 80-85° C. until the chlorine content is 50 per cent by weight of the composition, the chlorination being followed by specific gravity readings. The chlorinated naphtha is then blown with dry air at a maximum temperature of about 70° C. to remove dissolved HCl.

A charge consisting of 20 parts of the blown chlorinated naphtha, 12 parts of potassium ethyl xanthate and 35 parts by weight of dry acetone is then refluxed for two hours to obtain the crude reaction product which is washed at room temperature with 25 parts by weight of water, settled and the lower aqueous  $KCl$  layer drawn off. The supernatant layer containing the xanthate-chlornaphtha reaction product is then distilled at atmospheric pressure to remove the acetone. Residual acetone and water are removed by completing the distillation in a vacuum of 25-50 mm. at a maximum pot temperature of 90° C. The water-acetone-free product is then cooled and filtered to give the finished product, using Attapulgus clay as a filter aid. The acetone may be recovered for re-use in the process by careful fractionation.

It is to be understood that while we have herein described, for purposes of illustration, certain preferred examples of our reaction products with procedures for synthesizing same, the invention is not limited by the specific examples given but includes within the scope of products and procedures such changes or modifications as fairly come within the spirit of the appended claims, and it is further emphasized that while we have

stressed the value of these products as improving agents for lubricants, the present invention is directed to the products per se irrespective of the field in which they may find application.

We claim:

1. As a new composition of matter, the reaction product obtained by chemically substituting a part only of the chlorine in a chlorinated aliphatic hydrocarbon with a thiocarbonate group.

2. As a new composition of matter, the reaction product obtained by chemically substituting a part only of the chlorine in a chlorinated aliphatic hydrocarbon with a xanthate group.

3. As a new composition of matter, the reaction product obtained by chemically substituting a part only of the chlorine in a chlorinated aliphatic hydrocarbon with a trithiocarbonate group.

4. As a new composition of matter, a poly-chlorinated aliphatic hydrocarbon having from about five to about fifteen carbon atoms in which a part only of the chlorine has been chemically substituted with a thiocarbonate group, said product having a chlorine content of from about twenty-five to about forty per cent and a characterizing thiocarbonate group content of from about seven per cent to about twenty-two per cent.

5. As a new composition of matter, a poly-chlorinated aliphatic hydrocarbon having from about five to about fifteen carbon atoms in which a part only of the chlorine has been chemically substituted with a xanthate group, said product having a chlorine content of from about twenty-five to about forty per cent and a characterizing xanthate group content of from about ten per cent to about twenty-two per cent.

6. As a new composition of matter, a poly-chlorinated aliphatic hydrocarbon having from about five to about fifteen carbon atoms in which a part only of the chlorine has been chemically substituted with a trithiocarbonate group, said product having a chlorine content of from about twenty-five to about forty per cent and a characterizing trithiocarbonate group content of from about seven per cent to about seventeen per cent.

7. As a new composition of matter, a chlorinated petroleum naphtha in which a part only of the chlorine has been chemically substituted with a thiocarbonate group, said product having a chlorine content of from about twenty-five per cent to about forty per cent and a characterizing thiocarbonate group content of from about seven per cent to about twenty-two per cent.

8. As a new composition of matter, a chlorinated petroleum naphtha in which a part only of the chlorine has been chemically substituted with a xanthate group, said product having a chlorine content of from about twenty-five per cent to about forty per cent and a characterizing xanthate group content of from about ten per cent to about twenty-two per cent.

9. As a new composition of matter, a chlorinated petroleum naphtha in which a part only of the chlorine has been chemically substituted with a trithiocarbonate group, said product having a chlorine content of from about twenty-five per cent to about forty per cent and a characterizing trithiocarbonate group content of from about seven per cent to about seventeen per cent.

10. As a new composition of matter, the product obtained by reacting a poly-chlorinated aliphatic hydrocarbon with an alkali alkyl thiocarbonate in such proportions that only part of the chlorine in the aliphatic material is replaced by alkyl thiocarbonate groups.

11. As a new composition of matter, the prod-

uct obtained by: reacting chlorinated petroleum naphtha of from about forty per cent to about sixty per cent chlorine content and an alkali alkyl thiocarbonate in the ratio of about fifty to 5 seventy parts by weight of the thiocarbonate to about one hundred parts of chlorinated naphtha; and removing from the reaction mixture the alkali chloride formed.

12. As a new composition of matter, the product obtained by: reacting chlorinated petroleum naphtha of from about forty per cent to about sixty per cent chlorine content and an alkali alkyl xanthate in the ratio of about fifty to seventy parts by weight of the xanthate to about one hundred parts of chlorinated naphtha; and removing from the reaction mixture the alkali chloride formed.

13. The method of preparing a product adapted for use in extreme pressure lubricants and the like which comprises: chlorinating petroleum naphtha to a chlorine content of from about forty per cent to about sixty per cent by weight; dissolving said chlorinated naphtha in a solvent wherein alkali chlorides have low solubility; admixing with the solution thus formed a quantity of alkali alkyl thiocarbonate corresponding to from about forty per cent to about seventy per cent of the weight of chlorinated naphtha therein; boiling the reaction mixture under reflux to form a substitution product containing both chlorine and the alkyl thiocarbonate group in chemical combination with the naphtha; and separating alkali chloride from said substitution product.

14. The method of preparing a product adapted for use in extreme pressure lubricants and the like which comprises: chlorinating petroleum naphtha to a chlorine content of from about forty per cent to about sixty per cent by weight; dissolving said chlorinated naphtha in acetone; admixing with the solution thus formed a quantity of alkali alkyl thiocarbonate corresponding to from about forty per cent to about seventy per cent of the weight of chlorinated naphtha therein; boiling the reaction mixture under reflux to form a substitution product containing both chlorine and the alkyl thiocarbonate group in chemical combination with the naphtha; and separating alkali chloride from said substitution product.

50 15. The method of preparing a product adapted

for use in extreme pressure lubricants and the like which comprises: chlorinating petroleum naphtha to a chlorine content of from about forty per cent to about sixty per cent by weight; dissolving the chlorinated naphtha in acetone; admixing with the solution thus formed a quantity of alkali alkyl xanthate corresponding to from about forty to seventy per cent of the weight of the chlorinated naphtha; refluxing the mixture with stirring to form a substitution product containing both chlorine and alkyl xanthate groups in chemical combination with the characterizing hydrocarbon group of the naphtha; filtering the reaction mixture to remove alkali chlorides; and distilling the filtrate to remove the acetone.

10 16. The method of preparing a product adapted for use in extreme pressure lubricants and the like which comprises: chlorinating petroleum naphtha to a chlorine content of from about forty per cent to about sixty per cent by weight; 15 dissolving the chlorinated naphtha in acetone; admixing with the solution thus formed a quantity of alkali alkyl trithiocarbonate corresponding to from about forty to seventy per cent of the weight of the chlorinated naphtha; refluxing the mixture with stirring to form a substitution product containing both chlorine and alkyl trithiocarbonate groups in chemical combination with the characterizing hydrocarbon groups of the naphtha; filtering the reaction mixture to remove alkali chloride; and distilling the filtrate to remove the acetone.

20 17. The method of preparing a product adapted for use in extreme pressure lubricants and the like which comprises: chlorinating petroleum naphtha to a chlorine content of from about forty per cent to about sixty per cent by weight; dissolving the chlorinated naphtha in acetone; admixing with the solution thus formed a quantity of alkali alkyl thiocarbonate corresponding to from 25 about forty to seventy per cent of the weight of the chlorinated naphtha; refluxing the mixture with stirring to form a substitution product containing both chlorine and alkyl thiocarbonate groups in chemical combination with the characterizing 30 hydrocarbon groups of the naphtha; filtering the reaction mixture to remove alkali chloride; and distilling the filtrate to remove the acetone.

HENRY G. BERGER.  
ROBERT C. MORAN. 35  
FRANCIS M. SEGER. 50